

Oct. 24, 1950

G. W. SCOTT, JR.

2,526,698

METHOD AND APPARATUS FOR DIELECTRIC HEATING

Filed June 21, 1946

2 Sheets-Sheet 1

*Fig. 1.*



INVENTOR:

George W. Scott, Jr.  
by  
Stebbins, Blenks & Webb  
ATTORNEYS.

Oct. 24, 1950

G. W. SCOTT, JR

2,526,698

METHOD AND APPARATUS FOR DIELECTRIC HEATING

Filed June 21, 1946

2 Sheets-Sheet 2

**Fig. 2.**



**Fig. 3.**



INVENTOR:

George W. Scott, Jr.

by  
Stebbins, Blawie & Webb

ATTORNEYS.

## UNITED STATES PATENT OFFICE

2,526,698

## METHOD AND APPARATUS FOR DIELECTRIC HEATING

George W. Scott, Jr., Lancaster, Pa., assignor to Armstrong Cork Company, Lancaster, Pa., a corporation of Pennsylvania

Application June 21, 1946, Serial No. 678,215

15 Claims. (Cl. 18—5)

1.

This invention relates to the heating of electrical insulating material by the dielectric effect and, in particular, to a container or mold for confining insulating material in the form of loose particles during such heating in which the charge of material and the mold are both heated simultaneously by the dielectric effect.

The heating of various materials by the dielectric effect has come into extensive use in recent years. When the material to be heated is in the form of large solid masses, e. g., laminated wood board, little or no difficulty is encountered in maintaining it in proper relation to the spaced electrodes by which the high-frequency electric field is applied. A different situation prevails, however, in the case of material in the form of loose particles of small size which flow rather freely, such as cork granules lightly coated with a heat-activatable binder. In order to process such material into a solid block by dielectric heating, they must necessarily be confined since pressure must be applied to produce a cured mass of the desired density. No commercially satisfactory mold has been available heretofore for confining loose particles under pressure during processing by dielectric heating and it is the object of my invention to provide such a mold.

The characteristics desired in a mold for use in processing material by dielectric heating are well known but, so far as I am aware, no known construction of mold possesses sufficient of these characteristics to make it satisfactory for commercial production. In the first place, the mold walls must have high electrical insulating value to withstand the voltage applied across the electrodes between which the material to be heated is disposed. The mold walls must also have considerable mechanical strength, not only to withstand the pressure applied to the material during processing but also the relatively rough usage to which any apparatus involved in factory production is always subjected. In addition, the material used in the construction of the mold should be easily machinable to facilitate fabrication.

Wood naturally suggests itself as a material for mold walls capable of meeting these requirements but experience has shown that it also has shortcomings which make it quite unsuitable for the purpose. Even the densest woods are porous to a degree and contain more or less moisture. Although wood can be dried out quite thoroughly by appropriate treatment, it re-absorbs moisture from the atmosphere, because of its cellular structure, or from the material being processed if

it contains moisture. The amount of moisture present in wood, furthermore, varies from day to day with atmospheric conditions. This causes variations in the loss factor which is a measure of the likelihood of heat being generated internally when the wood is subjected to an electric field of a given voltage alternating at a given frequency. To be acceptable commercially, the material forming the walls of a mold for dielectric processing must have a loss factor within relatively narrow limits. If the factor is too high, an excessive amount of heat will be generated in the walls, resulting in a waste of electrical energy and possibly in injury to the walls themselves. If the factor is too low, the heat generated in the mold wall is not sufficient to bring its temperature up to that which is desired in the mass of material under treatment with the result that the mold wall cools the lateral surface of the mass. A further objection to wood for mold walls is that such moisture as is absorbed thereby is vaporized under the heat generated in the processing of the material to be treated, causing the wood to warp, split, crack or check and impairing or destroying its usefulness. In addition, wood mold walls, because of the absorbed moisture present therein, are susceptible to arcing which leaves carbonized paths through them and reduces their insulation value. For the foregoing reasons, wood as such has been abandoned, despite its apparent desirability, as a material for the walls of a mold for dielectric processing. Other materials such as ceramics and volcanic ash have been tried but without such success as to indicate any prospect of commercial adoption.

I have discovered that a highly satisfactory mold for dielectric processing may be made from hard wood which has been impregnated with a wax having special properties. Specifically, I employ ceresin or its equivalent as the impregnant for mold walls of hard wood such as maple, elm, birch, beech, oak or hickory. Other waxes having similar qualities, or a mixture thereof with ceresin, may also be employed. A mold constructed according to my invention has high insulation value at all temperatures encountered in curing heat-activatable mixes, a proper loss factor, is moisture-free and uniformly resistant to absorption, regardless of varying atmospheric conditions, and is not subject to warping or distortion on repeated heating and cooling. The impregnant is non-volatile, non-arcing and has a melting point high enough so that it does not "sweat" out of the wood under the temperatures involved in normal processing operations.

For a complete understanding of the invention, reference is made to the accompanying drawings illustrating a preferred embodiment and to the following description and explanation. In the drawings,

Figure 1 is a perspective view of a mold embodying my invention;

Figure 2 is a transverse section therethrough; and

Figure 3 is a circuit diagram.

Referring in detail to the drawings, a mold according to my invention comprises a box 10 open at the top and bottom and having side walls 11 of impregnated hard wood. As shown, the side walls 11 are preferably disposed with the grain thereof vertical. While the mold has been shown as of rectangular or square shape in plan, it may be of any other desired shape. The side walls 11 are secured in assembled relation by any suitable means, conveniently angle iron frames 12 and 13 at the top and bottom of the mold. These frames are composed of suitable lengths of angle iron welded together. The side walls are secured to the frames by wood screws 14 extending through the latter and into the former.

The mold 10 is adapted to confine a charge of material 15 during processing by dielectric heating. The charge may, for example, be cork granules coated with a glue-glycerine binder, a resin binder, latex, or the like adapted to be activated or cured by heat and converted into a solid mass. A plate 16 serves as a bottom for the mold. It rests on transverse pins 17 removably inserted through holes in opposite sides of the mold and the frame 13. For filling the mold with the charge, I employ a "boot" removably disposed on top of the mold, since the volume of the material when charged is considerably greater than when compressed within the mold for heating by the dielectric effect. The charge is compressed by applying pressure to a top plate 18 similar to the plate 16, disposed on top of the charge, and forcing it downwardly through the boot and into the mold to its final position in which it is held by pins 19 removably inserted through holes in the opposite side walls and the frame 12, in the same manner as the pins 17. The plates 16 and 18 serve not only as the bottom and top of the mold for confining the charge under pressure but also as condenser electrodes, having connections 20 to a suitable source of high-frequency alternating current.

The current source is a conventional electronic oscillator delivering a frequency of about 10 megacycles and a voltage of about 1.0 kilovolt per inch of thickness of the charge 15 when compressed to final volume.

The mold is provided with upper and lower peripheral conductors 21 connected to the plates 18 and 16, respectively, by straps 22 and 23 secured to the frames 12 and 13. The conductors 21 cause the portions of the charge adjacent the lateral surfaces to be heated to a temperature higher than that attained by the interior of the mass to compensate for the cooling effect to which the lateral portions are subjected.

The mold as described so far is also disclosed and claimed in my copending application, Serial No. 678,214 filed June 21, 1946 for Dielectric Heating Method and Apparatus.

The side walls 11 of the mold are composed of hard wood, such as maple, birch, beech, hickory, oak or elm, which should be straight-grained and free of knots or other irregularities. As previously stated, the pieces composing the side

walls are preferably disposed with their grain extending vertically. The boards from which the pieces are cut should not be heart wood. In making the mold, the pieces are thoroughly dried to reduce the moisture content thereof as low as possible. The pieces are then subjected to vacuum impregnation in a bath of a wax of suitable characteristics, heated to a temperature materially above its melting point and preferably in the neighborhood of, but below, its boiling point. The wood being practically bone dry is thoroughly impregnated by the wax and any residual moisture is vaporized and displaced. The wood pieces are left immersed for a sufficient time to insure thorough impregnation. After such time has elapsed, the pieces are removed, drained and, after cooling and solidification of the impregnated wax, they may be assembled into a mold as shown in the drawings.

The wax employed for impregnating the wood mold walls may be any one of a number of compounds. I have found, however, that ceresin has special properties which make it particularly desirable for this purpose. Ceresin or purified ozokerite, as it is sometimes called, is a white mineral wax which may be obtained with a melting point as high as 175° F. It is soluble in common hydrocarbons but is insoluble in water. It thus renders the impregnated side walls thoroughly water repellent, preventing any absorption of moisture either from the atmosphere or from the charge should it contain any moisture. Ceresin-impregnated wood when subjected to a high-frequency electric field, exhibits a relatively low loss factor, i. e.,  $K \tan \delta$ , where  $K$  is the dielectric constant and  $\tan \delta$  the dissipation factor. This expression may also be written as  $K \cos \theta$ , where  $\cos \theta$  is the power factor, if the latter is .1 or less. The actual values for ceresin are  $K$ , 2.14 and  $\tan \delta$ , .002 or less, at a frequency of 10 megacycles and room temperature, giving a loss factor of .004 or less. For maple wood impregnated with ceresin, the value for  $K$  is 2.8 and for  $\tan \delta$ , .042, at 10 megacycles and room temperature, giving a loss factor of .116. This value proves particularly desirable for the walls of a mold to be used in a particular practice of my invention, i. e., processing cork granules bonded with a mixture of glue and glycerin activated by paraformaldehyde (100 parts of cork, 6½ parts of glue, 20 parts of glycerin, 2½ parts of water and ½ part of formaldehyde, by weight). Such a loss factor is desirable because it avoids overheating the mold walls and the waste of energy incident thereto but is high enough to cause the mold walls to be heated to the proper temperature. Overheating of the mold walls might result in overcuring of the portions of the charge adjacent the lateral surfaces and perhaps in charring of the wood itself. The loss factor of ceresin-impregnated maple, .116, as given above, is less than that of the particular charge mentioned, viz., coated cork granules, which is 1.16 at 10 megacycles and room temperature. This is desirable in certain instances. In other cases, it may be desirable that the mold walls have a loss factor somewhat higher than the charge so they will not tend to exert a cooling effect on the latter. As an example, a maple 50 mold wall impregnated with Halowax 1012, chlorinated naphthalene, has a higher loss factor (.166) than a mass of phenol-formaldehyde molding powder having a filler of wood flour therein. This material has a loss factor of .156 at 10 megacycles and room temperature. Similarly, a urea-

formaldehyde molding powder having a cellulose filler has a loss factor of .12 under the same conditions.

A method of offsetting or preventing heat losses due to thermal conduction, convection, or radiation from the surface of a body of dielectric material to a mold wall, or the like, in which the mold wall has a higher loss factor than the body of dielectric material under treatment, is disclosed and claimed in the copending application of G. E. Gard, Serial No. 678,217, filed June 21, 1946, and entitled "Method of Compensation for or Preventing Heat Losses from Material During Dielectric Heating Thereof."

The following tables furnish data on the dielectric properties of a group of hard woods, impregnants, and hard woods impregnated with various impregnants.

Table I

| Wood <sup>1</sup> | Dielectric Values |              |             |
|-------------------|-------------------|--------------|-------------|
|                   | K                 | Tan $\delta$ | Loss Factor |
| Maple (dry)       | 2.5               | .064         | .16         |
| Maple (79% R. H.) | 6.2               | .088         | .55         |
| Maple (97% R. H.) | 9.2               | .162         | 1.49        |
| Oak (dry)         | 2.7               | .057         | .15         |
| Hickory (dry)     | 2.8               | .065         | .18         |
| Birch (dry)       | 2.6               | .052         | .14         |

<sup>1</sup> Measurements made with grain perpendicular to electrodes.

Table II

| Impregnant        | Melting Point in ° F. | Dielectric values |              |             |
|-------------------|-----------------------|-------------------|--------------|-------------|
|                   |                       | K                 | Tan $\delta$ | Loss Factor |
| Ceresin           | 130-175               | 2.14              | .002         | .004        |
| Paraffin          | 122                   | 2.08              | .003         | .006        |
| Beeswax and Rosin | 145-158               | 2.34              | .008-.010    | .019-.023   |
| Superla           | 165                   | 2.23              | .001-.003    | .002-.007   |
| Halowax 1012      | 203-210               | 3.38              | .034         | .115        |
| Halowax 1013      | 247-252               | 4.36              | .061         | .266        |
| Halowax 1014      | 277-283               | 3.84              | .048         | .184        |

Table III

| Mold material     |              | Dielectric values |              |             |
|-------------------|--------------|-------------------|--------------|-------------|
| Wood <sup>1</sup> | Impregnant   | K                 | Tan $\delta$ | Loss Factor |
| Maple (dry)       | Ceresin      | 2.84              | .042         | .116        |
| Maple (79% R. H.) | do           | 4.2               | .065         | .27         |
| Maple (dry)       | Paraffin     | 2.84              | .036         | .101        |
| do                | Superla      | 2.9               | .043         | .125        |
| Maple (97% R. H.) | do           | 5.0               | .057         | .29         |
| Maple (dry)       | Halowax 1012 | 3.2               | .051         | .166        |
| Maple (97% R. H.) | do           | 5.5               | .078         | .43         |

<sup>1</sup> Measurements made with grain perpendicular to electrodes.

All values for K, Tangent  $\delta$ , and Loss Factor were determined at a frequency of 10 megacycles with the material maintained at 70° F. Throughout this specification and in the claims the loss factor expressed is so determined. The Halowaxes are chlorinated naphthalene compounds and Superla is petroleum byproduct hydrocarbon wax.

As pointed out above, the optimum loss factor of a wax impregnated wood mold for cork composition manufacture is in the order of .116, and for best results, it is preferred to have the loss factor of the treated wood fall within the range of .1 to .25. It is possible, however, to utilize impregnated wood molds having a loss factor as

great as .4. For special molding operations, a loss factor somewhat above .4 may be desirable depending upon the geometry of the mold, the nature of the product being molded and heated, and other variable factors. Generally, however, a loss factor greater than .25 will not be necessary. By suitable combinations of wood and impregnant, or mixtures of impregnants, the desired loss factor may be obtained. For example, from Table I it may be determined that dry hickory has a loss factor of .18 and from Table II that Halowax 1013 has a loss factor of .266. By impregnating hickory with Halowax 1013, a mold wall having a loss factor between .20 and .25 may be obtained. It must be remembered that the use of an impregnant will increase the loss factor for any wood in dry condition, for the wood is constituted with considerable void space normally filled with air which is replaced by the impregnant which has a higher loss factor than air.

Tables I and III indicate clearly the effect of moisture on the loss factor of wooden mold materials. Maple wood, for example, maintained at 97% relative humidity for thirty days had a loss factor of 1.49 as contrasted with a loss factor of .16 for dry maple and .116 for ceresin impregnated maple. The loss factor of maple impregnated with ceresin and held at 79% relative humidity for thirty days is .27 and when impregnated with Superla and held at 97% relative humidity for the same time is .29, as contrasted with untreated maple held at the same relative humidities for equal times which has loss factors of .55 and 1.49, respectively.

Figure 3 shows how the mold is utilized in heating the charge. The electrode plates 16 and 18 are connected across a portion of a tuning coil 24 to which high-frequency alternating current is supplied from an oscillator indicated diagrammatically at 25. The charge between the plates is quickly heated by the dielectric effect as a result of the alternating electric field established between the plates. The heating effect is substantially uniform throughout the mass of material and it may thus be quickly brought to the temperature required for satisfactory curing of the heat-activatable binder, such as that mentioned above, resin, latex, or the like.

Experience has shown that a mold according to my invention provides a highly satisfactory solution for the problem of confining loose material during dielectric heating which is characterized by numerous advantages. In the first place, the side walls of the mold composed of hard wood thoroughly dried and impregnated with wax having the properties of ceresin, exhibit a high electrical insulation value and a low loss factor. As a result, the danger of overheating of the walls is minimized. The mold walls, furthermore, are characterized by electrical stability. The impregnant makes them uniformly moisture repellent so there is no substantial variation in the loss factor with normal atmospheric conditions. The high melting point of the wax and its lack of volatility prevent loss of impregnant from the wood during operation. The impregnant also renders the wood non-arcng so that the insulating property thereof is maintained indefinitely.

A mold with walls made in accordance with my invention is also characterized by mechanical stability. That is to say, the walls are not subject to warping, splitting or cracking as a result of the presence of moisture. The impregnating treatment vaporizes any residual moisture left in

the wood after drying and prevents the re-absorption of moisture from the atmosphere or the material being processed. The invention also provides mold walls which may be made at low cost and easily machined to provide the desired smooth surface with ample mechanical strength and toughness for the service to which the mold is subjected in use.

Although I have illustrated and described but a preferred embodiment of the invention, it will be recognized that changes in the details thereof may be made without departing from the spirit of the invention or the scope of the appended claims.

I claim:

1. In a method of forming molded articles the steps including depositing a charge of dielectric material in a mold composed of dielectric material having a loss factor between .1 and .4, and subjecting the material and mold to a high-frequency electric field for simultaneous heating by the dielectric effect.

2. In a method of forming molded articles the steps including depositing a charge of cork granules bonded with a mixture of glue, glycerin and para-formaldehyde in a mold of hard wood impregnated with ceresin and subjecting the granules and mold to a high-frequency electric field for simultaneous heating by the dielectric effect.

3. In a method of forming molded articles, the steps including: depositing a charge of cork granules coated with a heat-activatable binder into a mold composed of dielectric material having a loss factor between .1 and .4 and subjecting the material and mold to a high-frequency field for simultaneous heating by the dielectric effect.

4. In a method of forming molded articles, the steps including: compressing a charge of cork granules coated with a heat-activatable binder in a mold of hard wood impregnated with wax, said mold having a loss factor between .1 and .4, subjecting the material and mold to a high-frequency field for simultaneous heating by the dielectric effect, and continuing the application of said field until said binder has been activated.

5. In a method of forming molded articles, the steps including: depositing a charge of dielectric material to be molded into a mold composed of substantially moisture-free wood impregnated with a nonvolatile waterproofing impregnant substantially completely filling all of the void spaces within the wood and imparting to the mold a dielectric loss factor between .1 and .4 and subjecting the charge and the mold to a high-frequency field for simultaneous heating by the dielectric effect.

6. In a method of forming molded articles, the steps including: depositing a charge of cork granules coated with a heat-activatable binder into a mold of hard wood substantially free of moisture and substantially completely impregnated with a nonvolatile waterproofing impregnant, said mold having a loss factor between .1 and .25 and said charge having a substantially higher loss factor, and subjecting the charge and the mold to a high-frequency field for simultaneous heating by the dielectric effect to activate said binder.

7. In combination with a source of high-frequency current, a mold for confining a charge of dielectric material during processing by dielectric heating in which the charge of material and the mold are both dielectrically heated simultaneously, said mold comprising side walls of hard wood impregnated with a waterproofing impreg-

nant and having a loss factor between .1 and .4, and spaced electrodes connected to said source of high-frequency current and disposed to establish a high-frequency field in the mold and the charge for simultaneous heating of the mold and charge by the dielectric effect.

8. In combination with a source of high-frequency current, a mold for confining a charge of dielectric material during processing by dielectric heating in which the charge of material and the mold are both dielectrically heated simultaneously, said mold comprising side walls of hard wood substantially free of moisture and impregnated with ceresin, said mold walls having a loss factor between .1 and .4, and spaced electrodes connected to said source of high-frequency current and disposed to establish a high-frequency field in said mold and charge for simultaneous heating of the mold and the charge by the dielectric effect.

9. In combination with a source of high-frequency current, a mold for confining a charge of dielectric material during processing by dielectric heating in which the charge of material and the mold are both dielectrically heated simultaneously, said mold comprising side walls of hard wood substantially free of moisture and substantially completely impregnated with a wax, said mold walls having a loss factor between .1 and .4, and spaced electrodes connected to said source of high-frequency current and disposed to establish a high-frequency field in said mold and charge for simultaneous heating of the mold and charge by the dielectric effect.

10. In an apparatus for dielectric heating including a source of high-frequency current and a pair of spaced electrodes connected to said source; a mold for confining a charge of material disposed between said electrodes for processing by dielectric heating in which the charge of material and the mold are both dielectrically heated simultaneously, said mold comprising walls of hard wood substantially free of moisture and impregnated with a waterproofing material having a melting point above 130° F. which substantially completely fills all of the void space within the wood, said mold walls having a dielectric loss factor between .1 and .4.

11. In combination with a source of high-frequency current, a mold for confining a charge of dielectric material during processing by dielectric heating in which the charge of material and the mold are both dielectrically heated simultaneously, said mold comprising side walls of hard wood substantially free of moisture and substantially completely impregnated with a waterproofing impregnant of wax having a melting point above 165° F. and a loss factor between about .002 and .266 and imparting to the mold a dielectric loss factor between .1 and .4, and spaced electrodes connected to said source of high-frequency current and disposed to establish a high-frequency field in said mold and said charge for simultaneous heating of the mold and charge by the dielectric effect.

12. In combination with a source of high-frequency current, a mold for confining a charge of dielectric material during processing by dielectric heating in which the charge of material and the mold are both dielectrically heated simultaneously, said mold comprising side walls of hard wood substantially free of moisture and substantially completely impregnated with a waterproofing impregnant, said walls having a loss factor between .1 and .25, and spaced elec-

trodes connected to said source of high-frequency current and disposed to establish a high-frequency field in both said mold walls and charge for simultaneous heating of the mold and charge by the dielectric effect.

13. In combination with a source of high-frequency current, a mold for confining a charge of dielectric material during processing by dielectric heating in which the charge of material and the mold are both dielectrically heated simultaneously, said mold comprising side walls of maple substantially free of moisture and impregnated with a waterproofing impregnant consisting of ceresin having a melting point between 130 and 175° F. and a loss factor of .004 or less, said mold having a loss factor of about .116, and spaced electrodes connected to said source of high-frequency current disposed to establish a high-frequency field in said mold and charge for simultaneous heating of the mold and charge by the dielectric effect.

14. The combination of claim 7 in which the waterproofing impregnant is chlorinated naphthalene.

15. The combination of claim 7 in which the waterproofing impregnant is a hydrocarbon wax.

GEORGE W. SCOTT, JR.

#### REFERENCES CITED

The following references are of record in the file of this patent:

#### UNITED STATES PATENTS

| 10 | Number    | Name            | Date           |
|----|-----------|-----------------|----------------|
|    | 29,625    | Seiberling      | Aug. 14, 1860  |
|    | 1,377,241 | Winestock       | May 10, 1921   |
|    | 1,464,044 | Marr, Jr.       | Aug. 7, 1923   |
|    | 1,560,172 | Chamberlain     | Nov. 3, 1925   |
| 15 | 1,648,294 | Coolidge, 3rd   | Nov. 8, 1927   |
|    | 2,296,948 | Pitman          | Sept. 29, 1942 |
|    | 2,304,958 | Rouy            | Dec. 15, 1942  |
|    | 2,316,752 | Atkinson et al. | Apr. 20, 1943  |
|    | 2,322,903 | Wilkoff         | June 29, 1943  |
|    | 2,325,637 | Stewart         | Aug. 3, 1943   |
|    | 2,341,617 | Hull            | Feb. 15, 1944  |
|    | 2,421,097 | Lakso           | May 27, 1947   |
|    | 2,421,098 | Vogt et al.     | May 27, 1947   |